

# UNITED STATES PATENT OFFICE.

ENOCH OSGOOD, OF BOSTON, MASSACHUSETTS.

## IMPROVEMENT IN COMPOUNDS FOR PREVENTING THE DESTRUCTION OR ROTTING OF BAGS, &c.

Specification forming part of Letters Patent No. **216,290**, dated June 10, 1879; application filed May 8, 1879.

*To all whom it may concern:*

Be it known that I, ENOCH OSGOOD, of Boston, county of Suffolk and State of Massachusetts, have invented a new and useful improvement in a compound that will prevent the destruction or rotting of bags or other articles by acid phosphate, guano, alkaline matter, or any other article that will be destructive to textile articles, or bags made and used for the purpose of storing or transporting such articles, and that the following is a clear and full description of the same.

In describing the making and use of my compound, I first take (to illustrate the quantity, which can be varied as the case may require) bees-wax, three ounces; then add four ounces, more or less, of beef-tallow, (any tallow will do, but not as good;) melt and mix them well together. This will form a compound that will resist any acid, alkali, acid phosphate, or guano, and will protect acid phosphate and guano bags from rotting or injury while such articles are stored or transported.

To render this compound soft or plastic, in order to apply it to articles so that it will stick and not peel off, many things can be used, as oil, pitch, &c.; but for a safe, sure, and cheap article, take three ounces (more or less) of common tar, which add to the compound, melt all together, and when boiling or sufficiently hot, dip the bags or other articles into the compound until thoroughly saturated, take them out, and pass them through between two pressure-rolls, let them cool and they are ready for use.

I do not claim the coating of bags with tar, pitch, or gum, or crude petroleum-oil, or other oils, as specified and patented November 23,

1869, by Benj. Rowland Croasdale, nor do I claim a compound made as a water-proof mixture, of rosin, with tallow or oil, and rolled on when warm, as specified and patented March 5, 1872, and July 28, 1874, by said Croasdale, of hydrate of lime, oil, or mixed oil and paraffine.

As my invention, I use bees-wax, tallow, and common tar combined, or bees-wax and tallow combined, or either beeswax or tallow separately combined with tar, for the protection of bags and other articles against the destruction or rotting by acid phosphate, guano, &c., in their transportation or on storage, as herein specified.

The above-named compound is not unlike wax when applied to thread, giving strength to whatever it is applied, rendering it air and water tight, and preventing all smell and fine powder from escaping.

Having thus described my invention, what I claim, and desire to secure by Letters Patent, is—

1. A compound made of bees-wax and tallow melted together and applied to any article to prevent it from being destroyed or rotated by acid phosphate, guano, or any alkaline matter, substantially as and for the purposes herein set forth.

2. The combination of bees-wax and tallow, or either separately, with tar, as herein specified, and for the purposes substantially as herein set forth.

ENOCH OSGOOD.

Witnesses:

GEO. M. LOCKWOOD,  
JNO. H. SMALLWOOD.